

## UNITED STATES PATENT OFFICE

EARL EHRHARDT, OF CHICAGO, ILLINOIS

## COMPOSITION FOR ACOUSTICAL DEVICES

No Drawing.

Application filed May 18, 1928. Serial No. 278,922.

The present invention relates to compositions of matter or the like for acoustical devices, such as sound reproducers, reflectors, directors, conductors and radiators.

5 Among the objects of the invention is to provide a novel composition which may be plastic sufficiently long to shape or form the same into a desired or predetermined object, which when hardened is useful as a sound 10 radiator, reproducer, reflector, conductor, director or other like and similar objects, whereby the rendition of sound will be so true and faithful to the original natural sound that distinction between the two can 15 not be detected.

In acoustical devices, such as sound horns, reproducers, air column speakers, and even those of the hardened plastic type, there is generally the disadvantage of absorption of 20 certain parts of the sound, such as the harmonics, thus leaving the fundamental only to pass with a resultant unnatural rendition. Usually also, the emitted sound proceeds with a hollow or cistern 25 noise or sound; in some cases the sound is muffled; in some there is a resonance peculiar to the material used in the device, which resonance or foreign vibrations are parasitic to the sound reproduced, hence effecting 30 again an unnatural and false result; and in some the sound seems to proceed from a hard surface and is often termed as a hard sound. In all such cases the reproduced sound is not 35 pleasant; is far from being like the original sound being reproduced.

It is therefore an object of the invention to produce a sound device of a composition or material having the properties and characteristics to avoid and eliminate all of the disadvantages mentioned, such that the device 40 will be inert or dead so that sound cannot be transmitted therethrough nor absorbed thereby; nor dissipated in vibrating the material or resonating the same.

45 Another object is to provide a sound conducting, directing, reflecting or like surface which is preferably sufficiently rough, as by the presence of granular particles, such as sand and the like, for efficiently acting on the sound to prevent any loss of harmonics

or other qualities incident to the original sound being reproduced.

The composition also has the advantage of being fireproof, controllable in setting so that it may become hard and fully set in a few minutes or in a longer period, such as an hour or so as desired. It lends itself for use in trowelling, flow moulding, hand moulding and other like operations, whether for making the new object, patching or 55 plastering on a form, or the like. It is of such density and weight as not to absorb vibrations or to take up any vibration, and hence has no natural frequency of its own, but is 60 absolutely dead or inert. It makes a strong, 65 rigid and staunch article.

In the preferred illustrative use, it is applied to air column horns or loud speakers of the exponential form, yet is adapted for 70 sound devices, conduits and other like and similar sound or acoustical constructions.

The composition is preferably composed of prepared plaster, cement and plaster of Paris, with the addition of water or the like for making a plastic material which will 75 harden into the form given it. The prepared plaster usually comprises, plaster of Paris, sand or other like binding material, a retarder, and a small amount of hair. As an example, a prepared plaster having a composition of 33% of plaster of Paris, 33% of 80 screened torpedo sand, 1% of a retarder, and about one pound of hair per sack may be used to give good results. Such a prepared 85 plaster is prepared and sold by the U. S. Gypsum Company, of Chicago, Illinois, under the trade name "Big 4". The cement may be that such as known as Portland cement or the equivalent. Plaster of Paris is added to 90 act as a filler or consolidator, inasmuch as prepared plaster is more or less porous and by using a separate quantity of plaster of Paris, the composition as a whole, may be made more solid, compact or consolidated, or 95 more dense. Other material may be used in place of plaster of Paris, such as water putty, and other like and similar materials having the same characteristics as plaster of Paris, 100 for the purpose above mentioned. The ce-

ment is useful in aiding the hardening and setting of the composition.

The ingredients may be mixed in the proportions of about from 40 to 45% of prepared plaster, 50 to 60% of cement, and 5 to 15% of plaster of Paris and in some cases from 5 to 20%. Water may be added in any desired amount, which may be from 20 to 30% of the composition, but this water will, in the final composition, be substantially evaporated or dissipated, so that there is very little water included in the hardened product.

In a specific illustrative composition, the parts are mixed in the proportions of six parts by weight of cement, four parts of prepared plaster and one part of plaster of Paris. Each of these may be varied as desired. A sufficient amount of water is added to make the mixture plastic and control the time of setting. The proportions of the ingredients, when varied, will also vary the time of setting and hardening.

If the prepared plaster does not have a sufficient amount of sand for the purpose of this invention, sand may also be added in sufficient proportion to provide the desired roughened or granular surface whereby the sound will be properly guided, directed or reflected. By using the sand, a hard substance is formed in the surface, which will not absorb the sound qualities or harmonics, but which will bring out the fine qualities, while at the same time amplifying the sound, thus giving the naturalness to the reproduction and a faithful rendition of the original sound. By giving the surface a granular form, reflection of the smaller harmonics is made possible, whereas if a smooth or polished surface were used, only the fundamental sound would be reflected from such surface.

Cement aids in hardening the material so that it will be inert or dead and non-resonant.

The invention comprehends other characteristics, as will later appear and are inherently possessed thereby, and while I have herein disclosed an illustrative embodiment of the invention, it is to be understood that the latter is not limited thereto but may comprehend other features, ingredients, and the like without departing from the spirit thereof.

Having thus disclosed the invention, I claim:

A composition for acoustical devices comprising hardened plastic material containing grains of sand to render the surface rough.

In witness whereof, I hereunto subscribe my name to this specification.

**CERTIFICATE OF CORRECTION.**

Patent No. 1,905,631.

April 25, 1933.

**EARL EHRHARDT.**

It is hereby certified that error appears in the printed specification of the above numbered patent requiring correction as follows: Page 1, line 81, for "33%" second occurrence, read "66%"; and that the said Letters Patent should be read with this correction therein that the same may conform to the record of the case in the Patent Office.

Signed and sealed this 26th day of September, A. D. 1933.

**F. M. Hopkins**

(Seal)

**Acting Commissioner of Patents.**